

## UNITED STATES PATENT OFFICE

2,053,099

METHOD OF PRODUCING BITUMINOUS  
DISPERSIONS

Jack Miscal, Rutherford, N. J., assignor, by  
mesne assignments, to The Patent and Licens-  
ing Corporation, New York, N. Y., a corpora-  
tion of Massachusetts

No Drawing. Application July 26, 1932,  
Serial No. 624,911

8 Claims. (Cl. 134—1)

This invention relates to the production of dispersions of thermoplastic materials, and is particularly concerned with the production of soap-type dispersions by means of a colloid mill.

5 When a colloid mill is in operation, a great amount of air is sucked into the apparatus by reason of the vacuum created within the mill by the rapidly rotating parts. The air enters through the packing glands, bearing surfaces, 10 and through loosely connected joints.

In the production of soap-type dispersions of thermoplastic material such as asphalt in an aqueous medium, the presence of air is detrimental to the success of the operation. The air 15 causes a creaming effect with the result that a scum, containing a large proportion of poorly dispersed particles of asphalt, is formed. Additionally, when certain soaps, such as rosin soap, are used as the emulsifying agent, a chemical re- 20 action occurs between the soap and the carbon dioxide contained in the air. Rosin is composed chiefly of abietic acids which are weaker than carbonic acid and therefore displaced by the latter. The action of the carbonic acid on the soap 25 is accelerated at elevated temperatures and hence at the temperature at which the emulsion emerges from the colloid mill the reaction pro- 10ceeds fairly rapidly with the result that rosin is precipitated and the soap destroyed. As long as 10 the soap is present it acts as a protective colloid to maintain the large particles in suspension, but when it is precipitated the particles agglomerate into pellets which form a solid asphalt blanket on the emulsion. In addition, the incorporation 5 of air in the ingredients to be emulsified reduces the friction in the mill with the result that dispersion to the required degree is not effected. Furthermore, the incorporation of air greatly in- 15creases the volume of the ingredients passing through the mill,—sometimes as much as 40%,—so that the capacity of the mill is materially re- 20duced and the storage facilities must be greatly increased to handle the product.

The object of my invention is to provide means whereby to exclude air from the colloid mill during the emulsifying process.

Another object of my invention is to provide a method of producing soap-type emulsions of difficultly emulsifiable asphalts.

In accordance with my invention the colloid mill is immersed in a viscous liquid bath in order to prevent intake of air. A suitable liquid to be used as a bath is a heavy petroleum oil such as fuel oil or cylinder oil, but any other material that has sufficient viscosity so that it is not

easily sucked into the mill and at the same time is of such nature that it is not injurious to the emulsion when mixed therewith in small quantities, may be used as the bath.

In practicing my invention the materials to be dispersed are run into a colloid mill of the usual type such as a Hurrell mill and subjected to the emulsifying action of the mill. The feed to the mill is entirely closed and the mill itself is immersed in a receptacle filled with viscous oil or other viscous material, to a sufficient depth so that air cannot enter through the packing glands, bearing surfaces or through joints which ordinarily allow air to filter through. The dispersion then passes from the mill to a receptacle 15 where it may be tested and if found suitable, it is pumped to a storage tank. If the emulsion is unsatisfactory it may be recycled through the mill.

I have found that by using an oil bath for the 20 colloid mill it is possible to satisfactorily emulsify certain types of asphalt which it has heretofore been difficult or impossible to emulsify in the colloid mill which was exposed to the air, or 25 which produced poor emulsions when so emulsified. Not only has the quality of the dispersion been greatly improved but the volume of the emulsion has also been reduced more than 30% below that which is obtained when operating with the mill exposed to the air.

To illustrate my invention an emulsion was prepared with a Mexican type asphalt having the following specifications:

|                                       |                |    |
|---------------------------------------|----------------|----|
| Specific gravity                      | 1.01 to 1.03   | 35 |
| Softening point (B. & R.)             | 102 to 109° F. |    |
| Penetration (100 gr., 5 sec., 77° F.) | 180 to 210     |    |
| Ductility (77° F.)                    | 100            |    |
| Flash point                           | Over 450° F.   |    |
| Solubility in carbon bisulphide       | 99.8%          | 40 |

The asphalt was heated to 230° F. and proportioned through a colloid mill submerged in an oil bath, together with a rosin soap solution containing 25% excess potassium hydroxide over the amount necessary for saponification. The soap solution was heated to 80° F. The outlet temperature of the emulsion ranged between 160° F. and 180° F. The resulting emulsion contained 2.5% of soap and 42.5% of water. The emulsion was passed through a 28 mesh screen and showed 50 a screen deposit of only .016%. No scum was formed on the emulsion. An examination of the particles showed that none greater than 16 mu in size were present, while 70% were 4 mu or less.

The same asphalt heated to 240° F. was proportioned through a colloid mill, which was exposed to the air, together with a rosin soap solution containing 22% excess potassium hydroxide. 5 The emulsion issued from the outlet of the mill at a temperature ranging between 170° F. and 180° F. The water content was 43% and the proportion of soap present was 2.2%. The emulsion contained 25% to 35% of air by volume, gave a 10 very high screen deposit, and formed 2.2% of scum. An examination of the particle size showed 11.8% greater than 16 mu and 58% of 4 mu or less.

The emulsion prepared by using the oil immersed mill contained about 5% of air by volume, the source of which is not certain. However, the small amount of air present did not materially impair the quality of the emulsion.

With other types of asphalt than Mexican, the 20 effect of aeration is much more serious. With certain asphalts derived from Mid-Continent or Texas oils of semi-asphaltic nature, far greater liability to foaming or aeration is encountered. Apparently the surface tension relationships of 25 such asphalts vary greatly and a more permanent foam may result from aeration in the mill due to the character of the asphalt.

With certain asphalts derived from such oils 30 and having the same general melting point, penetration, and ductility characteristics as the Mexican asphalt referred to, the aeration is so severe that it becomes practically impossible to make a satisfactory emulsion at all in the ordinary type of colloid mill such as the Hurrell mill, in 35 which such aeration may come about.

With the above Mid-Continent asphalt, and using the same emulsifying agent as in the example given for Mexican asphalt, the emergent product from the mill when collected in a container is so heavily charged with air, and the 40 break-down occasioned thereby is so severe that a very substantial foam or crust forms on the emulsion. This foam or crust may be several inches thick on an ordinary 55 gallon barrel and 45 is a pasty, foamy mixture of air bubbles, aqueous phase, and agglomerated particles of asphalt, all in a condition which will not readily disperse into the better part of the emulsion, or if redistributed, re-collects. This foamy material 50 completely breaks down within a short time and the emulsion contained in this is, from a practical standpoint, unusable.

It is difficult to determine exactly why, under such conditions and with specific asphalts of this 55 kind, the effect of aeration should be so seriously destructive. One reasonable explanation, however, does reside in the fact that with asphalts having low surface tension relationship to air the foam produced in the severe action of the 60 mill is quite permanent. The air bubbles which are surrounded by the aqueous phase (with its

dispersed asphalt) being relatively permanent, may have the property of concentrating, on the surface or at the interface, by preferential adsorption, the soap which normally would be distributable about the asphalt particles. It is well 5 known that in the interfacial films of dispersions of this kind there is a concentration of the emulsifying media. Inasmuch as the air, as well as the asphalt, is the dispersed phase in a system of this kind, it will be seen that any preferential 10 adsorption of the emulsifying agent at the air-water interface would result in diminishing the stability of the dispersed asphalt while increasing the stability of the foam. The chemical effect 15 of the carbon dioxide in the aerated emulsion upon the soap, as hereinabove described, doubtless also contributes to the harmful results that ensue when emulsification is accompanied by aeration and the formation of foam. In running the same Mid-Continent asphalt as referred to above 20 in the mill, in which the feed is closed and in which the glands are sealed in a bath of oil, this aeration is practically eliminated and the emergent emulsion is substantially free from foam or 25 scum formation, being of normal particle size and free from coarse particles which produce screen residues, and is in every respect commercially usable.

I claim as my invention:

1. The process of emulsifying asphalt which comprises passing the molten asphalt through a colloid mill together with water and dispersing agent while said colloid mill is immersed in a liquid bath. 30
2. The process of emulsifying asphalt which comprises passing molten asphalt together with water and a dispersing agent through a colloid mill and preventing aeration during the emulsification, by the action of a liquid seal around the bearings of the mill. 35
3. In the process of producing soap type asphalt emulsions by colloid mill actions the step which comprises producing the emulsion in the substantial absence of air by the agency of a liquid seal around the bearings of the colloid mill. 40
4. The process of producing soap type asphalt emulsions which comprises passing asphalt in liquid state together with water and a soap-like dispersing agent through a colloid mill while said mill is immersed in a liquid bath. 50
5. Process in accordance with claim 4 in which the bath comprises a viscous oil. 55
6. In the production of asphalt emulsions by means of a colloid mill, the step of preventing access of air to said mill by immersing the mill in a liquid bath. 60
7. Method according to claim 6 in which the bath is composed of a viscous liquid.
8. Method according to claim 6 in which the liquid bath is a heavy hydrocarbon oil.

JACK MISCALL.